

## UNITED STATES PATENT OFFICE

1,948,906

## FLOWABLE COATING COMPOSITION

George Benjamin Dunford, St. Louis, Mo.

No Drawing. Application January 22, 1931  
Serial No. 510,509

9 Claims. (Cl. 134—51)

This invention relates to compositions of matter, such as binders and cements and more particularly to a bituminous binder which is useful for many purposes among which may be mentioned the lamination or building up of sheet material employed for building purposes. It is also useful as a deadening composition for deadening sound vibrations in relatively large expanses of metal such as in automobile bodies, 10 theater seats, ventilating systems and the like, as described in my copending application Serial No. 364,046 filed May 18, 1929, issued as Patent No. 1,914,912.

The so-called building or plaster board and 15 analogous sheeting of present manufacture takes many forms. Some of such sheeting consists merely of fibrous pulp formed as a sheet of convenient size, possibly one fourth of an inch thick; some manufacturers reinforce this by cementing 20 tough paper, such as kraft paper, to each surface of the sheeting, while still others place a waterproofing coating thereon. Some building board is constructed by forming a large sheet of plaster or mineral cement reinforcing it with fiber board 25 or paper cemented upon each side.

There has recently been developed a building board of wide application, which building board has been made possible by and includes my invention. This building board is constructed by 30 binding or laminating together a sheet of fiber board and a sheet of Portland or similar type of cement, preferably reinforced by fibers, the lamination being effected by the use of my novel binder and taking place preferably while the Portland cement sheet is in a moist, plastic, unset condition. A building board results which is not only 35 useful for inside partitions of buildings (as in the case of the other building board above mentioned), but which may be used as siding for buildings or shingles for roofs or similar uses wherein a permanent sheeting which will resist the elements is desired.

It is, therefore, among the objects of my invention to provide a composition of matter which is 40 useful for many purposes requiring a strong cementitious action but which is particularly useful in uniting a fibrous structure and wet plastic mass or for sound deadening purposes. Other objects will appear from a further perusal of this 45 specification.

Broadly, my composition comprises merely asphalt, a solvent for the asphalt, and talcous-agalite, together with a fiber such as asbestos. Although compositions of matter containing 50 these elements have been previously compounded,

my invention surpasses all such known compositions in that it comprises more specifically a mixture of selected asphalts with which is incorporated with the requisite special conditioning, a suitable solvent together with a tempering agent particularly appropriate for this type of composition. The talcous-agalite, together with fiber is then incorporated in this solution.

As an example of my invention, but by which I shall not, of course, be limited except as indicated by the claims appended hereto, the following is illustrative of the manner in which my novel binder is prepared. An asphalt mixture is first prepared by digesting in a steam jacketed mixing kettle approximately eleven parts, by 60 weight, of gilsonite asphalt having a melting point of about 275° F., about twenty-three parts of petroleum asphalt having a melting point of approximately 190°—200° F., about two parts of raw linseed oil, and approximately thirty-four to 65 thirty-five parts of ordinary varnish makers' and painters' naphtha having an initial boiling or distillation point of about 190° F. From this it will be observed that the ratio of the petroleum asphalt to gilsonite asphalt is approximately two 70 to one, and that the naphtha added is approximately equal to the total weight of asphalt.

The use of naphtha, or similar low-boiling, quick-evaporating hydrocarbon solvent in my composition is significant as it is by the use thereof that exceptional adhesive properties are obtained.

The naphtha above referred to may be either petroleum naphtha or coal tar naphtha. Other hydrocarbon solvents of this type which may be 80 employed are low-boiling petroleum distillate, benzine, benzol, toluol, and the like.

The foregoing ingredients are well mixed and digested at a temperature slightly below the boiling point of the naphtha in order that there will 85 not be too great evaporation of the naphtha. A temperature of approximately 185° F. has been found satisfactory. Obviously the mixing kettle is provided with adequate stirring means and is closed except for a small vent which is preferably provided with a condenser for recovering 90 any vapors issuing from the mixer, which may thus be saved or returned to the batch, all as will be apparent to those skilled in this art. The time of mixing is somewhat variable, according 95 to temperature, speed of stirring, etc., although it may be stated that with mild stirring a digesting and mixing time of one to four hours at about 185° F. is adequate.

The asphaltic solution so prepared may then 100

be drawn off and filtered or strained into an open type mixer and into it is then thoroughly incorporated approximately fifteen parts, by weight, of long fiber asbestos (such as the Canadian variety) and fifteen parts of talcous-agalite. After sufficient stirring to permit thorough penetration of the asbestos and talcous-agalite by the asphaltic solution, the binder is thus completed.

10 The talcous-agalite above referred to, and which I employ in my composition, is a talcous mineral, well known to mineralogists. It is largely composed of silicate of magnesia; the largest deposits thereof occur in northern New York in 15 St. Lawrence County. It has been mined in that locality and sold for forty years under the registered trade-mark "Asbestine", usually in the form of an impalpable powder. A representative sample thereof, has the following analysis:

|                               | Per cent |
|-------------------------------|----------|
| Silica                        | 61       |
| Magnesia                      | 31       |
| Lime (combined with silica)   | 4        |
| 25 Water (in crystallization) | 4        |

It is not to be confused with asbestos, which is of a fibrous character, nor with ground asbestos (sometimes loosely referred to in the trade as "Asbestine"), which likewise is of a fibrous character.

30 While it might at first be thought that the above composition would solidify upon cooling, the reverse is actually true, i. e. the composition remains flowable at all ordinary atmospheric temperatures and, it is found, can actually be sprayed with the ordinary type of air pressure spray gun so commonly employed in painting and lacquering. While asphaltic solutions are 35 ordinarily quite viscous and sticky, I have found that the "sprayability" of my binder is actually due to the presence of the asbestos and talcous-agalite or to the talcous-agalite alone which gives the requisite "slip" to the binder to pass 40 through the spray gun. The asbestos in my binder seems to have another important function in that when employed to bind layers of material containing moisture, the asbestos seems 45 to make the water compatible with the binder in a way which permits the binder to exert its tenacity toward a sheet even though the latter contains a considerable percentage of water; doubtless, the talcous-agalite also contributes 50 something in this regard as it seems to possess even more absorptive qualities than the asbestos; it also adds body to the composition. This 55 is indeed remarkable, as water is ordinarily not compatible with asphaltic solutions except when forming an emulsion—which obviously does not occur here. The asbestos also knits the binder together upon drying or hardening thereof.

60 The gilsonite asphalt toughens the composition, whereas the petroleum asphalt gives it the requisite body to withstand the higher atmospheric temperatures following evaporation of the naphtha from the binder upon use thereof. By proportioning these two asphalts as I have, I am able to obtain a binder of great utility. The 65 value of the raw linseed oil in my binder is also not to be overlooked. By digesting the asphalts in the raw linseed oil, the asphalts are thus tempered so that embrittlement of the asphalts upon 70 hardening of the binder is avoided. The presence of the linseed oil in the binder also seems to have a plasticizing effect upon the binder so

as to induce flexibility, tenacity, and tensile strength to the hardened binder.

75 In the preparation of the building board above described the fiber board is laid upon a press and my binder is coated thereon to a thickness of approximately one sixteenth of an inch. It may be either sprayed on or spread on with a trowel, brush or the like. A damp and plastic sheet composed of Portland or similar cement, water and some form of fiber, of the desired thickness 80 is then laid upon the binder. A steel sheet separates these sheets from further laminations which are built up so that a pile three or four feet high 85 results. This pile is then pressed at several hundred pounds pressure—say 500 pounds per square inch—and permitted to stand at that pressure until the Portland cement has taken an initial set. One hour is about sufficient. Upon removal of the pressure, the resulting boards may be oven cured or permitted to cure in stacks in ordinary 90 atmosphere for a while.

95 When the sheet has cured, it will be found that the hardened Portland cement lamination adheres firmly to the fiber sheet and that the resulting building board appears to consist of a homogeneously merged fiber and cementitious structure which will withstand the ordinary elements with an unusual degree of excellence. Examination of such board will disclose that my binder has so completely merged or coalesced with the 100 cement lamination that the two are substantially homogeneous, and also that my binder has penetrated the fibers of the fiber board to an extent sufficient for it to encase and grip the fibers to 105 tenaciously unite the two laminations.

110 Obviously the cement sheets may be placed upon both sides of the fiber sheet by coating my binder upon each side of the fiber sheet and pressing the cement sheet therewith. Furthermore, numerous other uses for my binder than 115 that described above will occur to those skilled in the art and the foregoing is to be understood as merely illustrative of the uses to which my invention may be put.

120 In addition, there will also occur to those skilled in the art many variations in the proportions of constituents in my binder and the method of preparing it. For instance, the proportion of petroleum asphalt to gilsonite asphalt may be varied slightly above or below the ratio of two to one. 125 The amount of naphtha may be varied somewhat, it being obvious that a thicker or thinner binder will result from decreasing or increasing, respectively, the amount of naphtha employed. The beneficial effect of the raw linseed oil may also be 130 varied within reasonable limits by varying the amount of linseed oil employed, although it will be understood that the proportion given results in an excellent binder and that the ratio of this tempering agent should not be greatly changed, if the 135 best results are desired. The proportion of asbestos and of talcous-agalite may also be varied somewhat to make a more or less plastic binder or for some purposes one may even be omitted, although for the purpose described, the asbestos 140 has an important function, as above mentioned, as does also the talcous-agalite, the latter giving "slip" to the composition which permits it to be sprayed onto the work; if one of these is to be omitted, it would be preferable to retain the 145 talcous-agalite in the composition because of its superior absorptive and "slip" giving properties.

What I claim as my invention and desire to be secured by Letters Patent of the United States is:

1. A coating composition which is flowable at 150

- atmospheric temperatures and which comprises approximately two parts asphalt, a quantity of naphtha at least equivalent to the weight of the asphalt, and at least one part talcous-agalite.
5. 2. A coating composition which is flowable at atmospheric temperatures and which comprises approximately two parts asphalt, a quantity of a low-boiling, quick-evaporating hydrocarbon solvent for the asphalt at least equivalent to the weight of the asphalt, and at least one part talcous-agalite.
10. 3. A coating composition which is flowable at atmospheric temperatures and which comprises approximately two parts asphalt, a quantity of a low-boiling, quick-evaporating hydrocarbon solvent for the asphalt at least equivalent to the weight of the asphalt, and at least one part of a non-fibrous talcous mineral which contains approximately 92 percent silicate of magnesia and an appreciable percentage of lime.
15. 4. A coating composition which is flowable at atmospheric temperatures and which comprises approximately two parts asphalt, a quantity of naphtha at least equivalent to the weight of the asphalt, at least one part talcous-agalite, and at least one part of asbestos.
20. 5. A coating composition which is flowable at atmospheric temperatures and which comprises approximately two parts asphalt, a quantity of a low-boiling, quick-evaporating hydrocarbon
- solvent for the asphalt at least equivalent to the weight of the asphalt, at least one part talcous-agalite, and at least one part of asbestos.
6. A flowable coating composition comprising in approximate parts by weight the following: thirty-four parts asphalt, at least thirty-four parts naphtha, and at least fifteen parts talcous-agalite.
80. 7. A flowable coating composition comprising in approximate parts by weight the following: eleven parts gilsonite asphalt, twenty-three parts petroleum asphalt, two parts linseed oil, thirty-four parts naphtha, fifteen parts asbestos, and fifteen parts talcous-agalite.
85. 8. A flowable coating composition comprising in approximate parts by weight the following: eleven parts gilsonite asphalt, having a melting point of about 275° F., twenty-three parts petroleum asphalt, having a melting point of 190°-200° F., two parts linseed oil, thirty-four parts naphtha, and fifteen parts talcous-agalite.
90. 9. A flowable coating composition comprising in approximate parts by weight the following: eleven parts gilsonite asphalt, having a melting point of about 275° F., twenty-three parts petroleum asphalt, having a melting point of 190°-200° F., two parts linseed oil, at least thirty-four parts low boiling naphtha, fifteen parts asbestos, and at least fifteen parts talcous-agalite.

GEORGE BENJAMIN DUNFORD. 105

35. 110

40. 115

45. 120

50. 125

55. 130

60. 135

65. 140

70. 145

75. 150